

## UNITED STATES PATENT OFFICE

2,506,731

METHOD OF PREVENTING TARNISHING OF  
THE SURFACES OF SILVERWAREJames Clayton Moss, New York, N. Y., assignor  
to Celanese Corporation of America, a corpo-  
ration of DelawareNo Drawing. Application January 25, 1945,  
Serial No. 574,640

2 Claims. (CL 21—2.5)

1

This invention relates to the prevention of the tarnishing of the surfaces of metal articles, and relates more particularly to the prevention of the tarnishing of the surfaces of silverware.

The surfaces of silverware, i. e. silver or silver-plated articles, such as dishes, trays, coffee and tea sets, flatware and the like, are readily tarnished by exposure to the atmosphere, with the result that unsightly coatings appear thereon. To prevent the tarnishing of silverware, the pieces are normally covered with a napped, wool or cotton cloth such as flannel, treated or untreated, or placed in bags or sheets made of this material. However, such flannel coverings are not satisfactory since they prevent the tarnishing of the silverware surfaces for only a very short time. It is, accordingly, an important object of this invention to provide a novel method of preventing the tarnishing of silverware surfaces which will be particularly effective over a very long period of time.

Another object of this invention is the provision of an improved fabric covering for silverware which will prevent the tarnishing of the surfaces thereof for a substantially long period of time.

A further object of this invention is the provision of a fabric of relatively close construction and having a basis of an organic derivative of cellulose which when wrapped around silverware will prevent the tarnishing thereof over a substantially long period of time.

Other objects of this invention will appear from the following detailed description.

I have found that the tarnishing of silverware is effectively prevented over a substantial period of time by covering the same with a textile fabric, preferably of closely woven construction, made of or containing filaments, threads, yarns and the like having a basis of an organic derivative of cellulose.

In accordance with my invention, I cover the silverware with a woven textile or knitted textile fabric made of or containing filaments, threads or yarns having a basis of an organic derivative of cellulose, by wrapping the silverware in a piece of said fabric or by inserting the silverware in bags, envelopes or sheaths made from said fabric. I prefer, however, to employ a fabric of closely woven construction, i. e. having a satin, taffeta, or sharkskin weave. The silverware covered by such a fabric is tarnish-proof over a substantially long period of time.

Any suitable organic derivative of cellulose may be employed as the basis of the filaments,

20

threads or yarns from which the fabric employed in accordance with this invention is made. For instance, I may employ organic derivatives of cellulose such as organic esters of cellulose, or 5 cellulose ethers. Examples of organic derivatives of cellulose are cellulose acetate, cellulose propionate, or cellulose butyrate, while examples of cellulose ethers are ethyl cellulose and benzyl cellulose. Furthermore, mixed esters,

10 such as cellulose aceto-propionate and cellulose aceto-butyrate may be employed as the basis of the filamentary materials. However, we prefer to employ cellulose acetate filaments, threads or yarns, as cellulose acetate is commercially the 15 most important of the organic derivatives of cellulose employed at the present time.

As a means for illustrating my invention, but without being limited thereto, the following example is given:

## Example

25 A fabric is woven with a sharkskin weave 42" wide and weighing 5 ounces to the square yard. The warp yarns are 150 denier cellulose acetate yarns placed 116 ends per inch and the filling 30 yarns are 450 denier cellulose acetate yarns placed 44 picks per inch. This fabric may be cut into suitable lengths or sewn into bags, envelopes or sheaths for the purpose of placing silverware therein. Silverware covered with said 35 fabric showed no trace of tarnishing over a three-month period of time, whereas silverware covered with wool or cotton flannel showed considerable tarnishing after a period of only one month.

The term "silverware" as employed in the 40 claims is to be construed as including within its scope any metal articles capable of being tarnished by atmospheric conditions. The expression "closely woven construction" as employed in the claims is to be construed as meaning a satin, taffeta or sharkskin weave.

It is to be understood that the foregoing detailed description is given merely by way of 45 illustration and that many variations may be made therein without departing from the spirit of my invention.

Having described my invention, what I desire to secure by Letters Patent is:

1. A method of preventing tarnishing of the surfaces of silverware, which comprises placing said silverware in a covering shaped to receive said silverware, said covering comprising a fabric of closely woven construction containing filamentary materials having a basis of a lower aliphatic acid ester of cellulose.
2. A method of preventing tarnishing of the

55

surfaces of silverware, which comprises placing said silverware in a covering shaped to receive said silverware, said covering comprising a fabric of closely woven construction containing filamentary materials having a basis of cellulose acetate.

JAMES CLAYTON MOSS.

REFERENCES CITED

The following references are of record in the 10 file of this patent:

UNITED STATES PATENTS

| Number     | Name    | Date          |
|------------|---------|---------------|
| Re. 18,379 | Herring | Mar. 8, 1932  |
| 312,954    | Blain   | Feb. 24, 1885 |

OTHER REFERENCES

Fall and Winter Catalog of the Montgomery-Ward Co. for the Period 1941-1942. Copy identified as vol. 135.